

## UNITED STATES PATENT OFFICE

RALPH M. HUNTER AND SHELDON B. HEATH, OF MIDLAND, MICHIGAN, ASSIGNOR TO THE DOW CHEMICAL COMPANY, OF MIDLAND, MICHIGAN, A CORPORATION OF MICHIGAN

## METHOD OF MAKING METALLIC MAGNESIUM

No Drawing.

Application filed May 27, 1929. Serial No. 366,518.

The present invention concerns a method of producing metallic magnesium by the electrolysis of a fused bath containing magnesium chloride ( $MgCl_2$ ) and concerns more particularly the method of maintaining the bath by feeding to it a compound of magnesium.

In the electrolysis of such a fused bath wherein metallic magnesium is liberated and collects at the cathode and chlorine is liberated and drawn off at the anode, continuous operation is desirable and it becomes necessary to replenish the bath and maintain it of the desired character by feeding thereto an equivalent of the magnesium and chlorine or other essential ingredients which, in the course of operations, have been or may be removed therefrom.

It is well known that the ideal feed to such a cell comprises anhydrous  $MgCl_2$  and that accompanying water will reduce the current and power efficiency of electrolysis. It is further known that inert constituents of the feed, such as  $MgO$ , tend to settle out of the bath, and unless removed therefrom, will accumulate and interfere with continuous operation. Such sediment must accordingly be removed, which is customarily done by dredging from time to time as required, but this operation removes also part of the bath along with the sediment or so-called sludge. In practice we have found that as high as two equivalents of bath may be removed in that way with one equivalent of sludge figured as  $MgO$ . The bath so removed with the sludge must, of course, be returned by feeding to the cell the constituents so removed in addition to that required to replenish the  $MgCl_2$  converted to metal and chlorine.

Anhydrous  $MgCl_2$  is not only difficult and expensive to prepare, but on account of its hygroscopic properties it is practically impossible to handle it without its taking up some moisture, and in practice, a content of 95 per cent  $MgCl_2$  in the chloride fed to the cell is considered obtainable good practice. In U. S. Patent No. 1,567,318 is disclosed a method of feeding  $MgCl_2$  containing water, whereby the detrimental effects of the water are minimized.

In the copending application Serial No. 280,659, there is disclosed by Sheldon B. Heath, co-inventor herein, a method of utilizing magnesium chloride containing basic chloride to replenish and maintain the fused bath.

We have discovered an improved method of introducing the  $MgCl_2$  fed to such an electrolytic cell having marked advantage as contrasted with methods heretofore disclosed or known to us, said improved method being applicable to introduction of  $MgCl_2$  containing water or similar introduction of  $MgCl_2$  containing basic salt.

To the accomplishment of the foregoing and related ends, the invention, then, consists of the steps hereinafter fully described and particularly pointed out in the claim, the following description setting forth in detail one approved mode of carrying out our invention.

It has heretofore been customary to introduce the feed at one point in the cell and in accordance with the patent application referred to above, adjacent the anode. Such method of feeding gave improved results over previous practice on a relatively small scale, but when cells of large capacity were used, particularly cells employing a plurality of anodes which in certain cases may be distributed relative to a large bath area, that method of feeding was found to produce large quantities of sludge, to involve over-cooling of the bath locally at the point of feed introduction, and to localize anode wear. The removal of this excessive quantity of sludge entailed the removal therewith of increased quantities of bath requiring increased added feed to maintain the bath, such feed carrying with it more basic salt or water or both, thereby adding still further to the sludge formation.

We have now discovered that if the cell feed including  $MgCl_2$  containing basic salt or water or both be fed to the cell in a manner to distribute it relative to the active anode surface, a smaller amount of sludge is formed, local cooling of the bath is substantially avoided and the anode wear is distributed more evenly. The dredging is correspond-

ingly reduced as is the loss of bath therewith and what is most important the requirement for feed is likewise markedly reduced. The mechanics of the phenomenon of reduced sludge production are not definitely known. It may be that the distributed mode of feeding permits the solution in the bath of the basic chloride adjacent the active anode surface instead of allowing it to fall to the bottom of the bath where it becomes inert and that the so dissolved basic salt is reacted upon by CO and chlorine to form  $MgCl_2$ ,  $CO_2$  and  $HCl$ . Whatever the cause of the said phenomenon the improved method of introducing the feed constitutes a valuable improvement in the art.

A simple method of attaining distribution of the feed relative to the anode surface is to introduce said feed at a number of points instead of at one point. The size, character and form of the cell will naturally determine the exact method of introduction and the number of points at which introduction may advisably be made, but very marked improvement is attained by introducing at even but two points in a cell of upwards of 10000 ampere capacity and a still further improvement may be expected by introducing such feed at more than two points, the feed being introduced in a fairly continuous manner.

We have found further that good results may be thus obtained when using a feed carrying as low or lower than 5 per cent equivalent  $MgO$  by introducing it into the bath at other points than adjacent the anode, but we prefer, particularly with feeds running higher than 5 per cent equivalent  $MgO$  content, to introduce same adjacent the anode distributed relative to the anode surface.

Other modes of applying the principle of our invention may be employed instead of the one explained, change being made as regards the method herein disclosed, provided the step or steps stated by the following claim or the equivalent of such stated step or steps be employed.

We therefore particularly point out and distinctly claim as our invention:

In the production of metallic magnesium by electrolyzing a molten bath containing magnesium chloride, wherein the raw material fed to said bath consists of magnesium chloride containing some water or basic chloride, the improvement which consists in feeding such raw material to said bath adjacent the anode at a plurality of points distributed with reference to the anode surface.

Signed by us this 23rd day of May, 1929.

RALPH M. HUNTER.

SHELDON B. HEATH.